

No. 629,685.

Patented July 25, 1899.

C. HOEPFNER.

ELECTROLYTICAL PRODUCTION OF ZINC OR OTHER METALS.

(Application filed July 16, 1898.)

(No Model.)



Witnesses  
B. S. Ober.  
W. W. Summers

Inventor,  
Carl Hoepfner  
By Harry M. Dake

# UNITED STATES PATENT OFFICE.

CARL HOEPFNER, OF BERLIN, GERMANY.

## ELECTROLYTICAL PRODUCTION OF ZINC OR OTHER METALS.

SPECIFICATION forming part of Letters Patent No. 629,685, dated July 25, 1899.

Application filed July 16, 1896. Serial No. 599,442. (No specimens.)

To all whom it may concern:

Be it known that I, CARL HOEPFNER, a subject of the King of Prussia, Emperor of Germany, residing at No. 2 Helgoländer-Ufer, Berlin, Germany, have invented certain new and useful Improvements in the Electrolytical Production of Zinc or other Metals, (for which Letters Patent have been obtained in France, No. 250,075, dated September 5, 1895, and in Belgium, No. 117,278, dated September 5, 1895;) and I do hereby declare the following to be a clear and exact description of the invention.

This invention consists in improved methods for carrying out electrolytic decompositions in as rational and economical a manner as possible—*i. e.*, with the least possible electromotive force—especially such decompositions in which it is desired to obtain valuable products only—for example, where zinc or other metals, such as iron, nickel, or copper, are to be obtained from their salts by the electrolytic process at a moderate cost. I propose to employ a bath which for ordinary cases should be divided by suitable membranes or diaphragms into anode and cathode cells in such manner that all the cells of like name will be connected in series through suitable conduits, so that the electrolyte will circulate there-through in a zigzag manner, flowing into the first cell of a series of such at the bottom and flowing out of the last cell at top, or vice versa, any suitable means being provided for heating the electrolyte.

Apparatus such as referred to may be of any well-known construction—as, for instance, of the construction shown and described in my British Letters Patent No. 13,735 of 1890 or as shown in the accompanying drawings, in which—

Figure 1 is a horizontal section of an electrolytic apparatus or bath embodying the necessary conditions for carrying out my invention. Fig. 2 is a vertical transverse section of one form of anode, and Fig. 3 is a transverse section between two cell-frames of an apparatus such as shown in Fig. 1.

The cells are formed by a series of frames, of which I have shown eight, said frames being correspondingly numbered and are provided in their vertical members with passages or channels *x y z*, so arranged that when said

frames are clamped together between suitable heads *h h'* by means of the two rods *S* and clamping-bars or plates *P* the said channels 55 will connect the cells of like name in series, so that the electrolytes fed under suitable pressure to the anode and cathode cells will enter anode-cell 1 at top at *a*, rise therein, and flow through channels *x y z* to anode-cell 3, 60 thence flow through like channels on the inlet side of the apparatus to anode-cell 5, and so on zigzag fashion from one anode-cell to another, flowing out at the inlet side of the apparatus from bottom of cell 7 at *b*. The 65 electrolyte for the cathode-cells *K* follows a substantially similar course, entering at the top of first cathode-cell 2 at *c* and flowing from the bottom of the last cathode-cell 8 at *d*.

The electrolytes are preheated in any suitable manner and their temperature kept up during the flow through the respective cells by causing such electrolyte—as, for instance, the cathode-cell electrolyte—to flow from top of cell 1 to a branch *c'*, connected with one 75 of the terminals of a heater-coil at *C'*, and flowing back therefrom through a branch *c''*, connected with the other terminal of the coil *C'*, which latter is contained in a suitable heating-chamber *C<sup>2</sup>*, to which any desired 80 heating agent is supplied—as steam, for instance, entering at *e* and flowing out at *f*. A similar arrangement is or may be provided for heating the electrolyte for the cathode-cells or for maintaining the preheated electrolyte at the proper temperature. 85

*A* indicates the anodes, *K* the cathodes, and *M* the cell-diaphragms clamped between the cell-frames 2 3, &c.

The electrolyte or solution to be decomposed and supplied to the cathode-cells may, for example, be a solution of the metallic salt to be decomposed—such as chlorid of zinc, bromid of zinc, sulfate of zinc, nitrate of zinc, or acetate of zinc, or an alkaline solution of 90 oxid of zinc, or similar solutions of other metals—while the cathodes will consist of carbon or any suitable metal in the shape of plates, disks, rods, or hollow bodies. 95

It will be found very advantageous to actively maintain the cathode solution or lye at the cathodes in constant motion, for which purpose the cathodes are kept revolving or vibrating, and it is also necessary that the 100

lye should be sufficiently concentrated and kept warm and be made to circulate from an appropriate reservoir through the cell in a suitable manner.

5 The anodes I employ for the purpose of reducing the electromotive force required for decomposition to a minimum (in fact, for making it actually negative in the case of copper salts, for example) are not insoluble, 10 but are soluble anodes consisting of metals or metalloid substances, while I take care at the same time that the solutions obtained therefrom do not reach the cathodes, but are precipitated from the anode lye in a harmless 15 manner before they become too rich or abundant.

The metals dissolved from the anodes are in fact made insoluble either chemically or physically, (or, in other words, in any convenient manner,) and the resulting precipitates, which may be obtained within but should be preferably produced outside the anode-cell, are collected and utilized again for any useful purpose. As a rule they 25 should be reduced—*i.e.*, restored—to the metallic state by means of carbon or other reducing substances, such as hydrogen or water-gas, or by organic substances, as wood or coal.

The metal of the soluble anodes differs 30 from the metal of the final product to be obtained at the cathode and is readily precipitable from its solutions, (like lead,) but is insoluble in diluted acid, (especially in diluted sulfuric acid,) so as to exclude, for instance, 35 zinc and iron from the employment for the anodes. Such anodes, therefore, may preferably consist of lead or materials containing lead, such as sulfuret of lead or argentiferous lead. These materials may be employed in 40 the form of solid bars or plates or (especially in the case of sulfids) in a granulated or powdered condition, in which case the said material will be contained in a holder or casting of wire fabric *a'* or of perforated plates, 45 as shown in Fig. 2. In the latter case the electric current may be admitted through electronegative metals—such as gun-metal, or copper-bronze, or silver wire-netting, or carbon rods, or the like—which should be retained 50 in close contact with the pulverulent metals or sulfids. As to the anodes it is also better to keep them in motion, so as to facilitate the formation of a uniform solution and the employment of powdered sulfids, which 55 otherwise might lose the contact.

The anodes are surrounded by an acid or a salt solution, which should preferably be heated, and the nature of which should be such that it will readily dissolve the compounds of lead formed electrolytically at the anode. The agents most suitable for the attainment of this object are solutions of chlorids, such as common salt, chlorid of calcium, chlorid of zinc, chlorid of potassium, or the like, or, more conveniently, nitrates or nitrites, such as nitrate of sodium or nitrate of zinc, or acetates, such as acetate of sodium

or acetate of zinc, or acids or salts capable of forming soluble compounds with lead. In order to enable this process to be kept up in 70 a regular manner for a comparatively extended period of time, care must be taken to prevent the anode lye from absorbing too large an amount of lead—in no case more than from about fifty to one hundred grams per 75 liter—for if the quantity were larger it would cause the voltage necessary for the decomposition to rise unduly, besides the lead, or instead of lead other metals which are used for and dissolved from the anode, would be 80 readily diffused toward the cathode and thereby impair the purity of the zinc. The lye, therefore, constantly circulates past the anodes and is freed in the course of this process within or, which is still better, outside the 85 bath from the whole or part of the lead (or other metal) which it contains. For the purpose of this precipitation of the lead from the anode lye any useful chemical precipitant may be used which is from the point of view 90 of economy capable of precipitating lead from its solutions without introducing other injurious matters into the solution instead of such lead.

In obtaining zinc by this electrolytic process the following chemical agents will be found best suited for precipitating the lead from its solutions: sulfate of zinc, ( $ZnSO_4$ ), chromate of zinc, ( $ZnCrO_4$ ), sulfite of zinc, ( $ZnSO_3$ ), carbonate of zinc, ( $ZnCO_3$ ), silicate 100 of zinc, ( $ZnSiO_3$ ), oxid of zinc, ( $ZnO$ ), sulfid (or sulfuret) of zinc, ( $ZnS$ ), and chlorid of zinc, ( $ZnCl_2$ ). By means of any of these agents lead may be precipitated from solutions of chlorid, nitrate, or acetate in a very rational manner, 105 and at the same time (by alternate decomposition) the lye will again be enriched with zinc, the reaction being as follows:



Insoluble.

By means of pure oxid of zinc and carbonic acid white lead may be obtained. Instead of these zinc compounds where a cheaper solution of zinc is available and where, therefore, 115 a regeneration of the zinc solutions is not necessary other harmless precipitants may be utilized in precipitating the lead—such as alkaline chlorids, bromids, chromates, sulfates, sulfites, sulfids, or similar compounds with 120 alkaline earths, sulfureted hydrogen, ammonia, the alkaline earths themselves, carbonates, and sometimes acids, such as sulfurous or sulfuric acid and carbonic acid, and finally, also, oxid of lead, other lead compounds, such 125 as hydroxid or carbonate of lead or substances containing oxid of lead, such as roasted lead ores, which will form a nearly insoluble basic salt when brought into contact with the salt of lead contained in the anode lye. In some 130 cases—*i.e.*, where an inexpensive source of heat is available—the dissolved salt of lead may be precipitated simply by a physical process—viz., by cooling, by diluting the so-

lution, or by the addition of an acid. In order to reliably prevent a diffusion of lead from the anodes to the cathodes, sulfates or other substances capable of rendering the salts of lead insoluble may be added to the circulating cathode lye outside or inside the bath.

The lead compounds—such as sulfate of lead, chlorid of lead, oxid of lead, or sulfid of lead—precipitated in the manner hereinbefore described and which, as above explained, may vary extensively in their nature may be utilized in any convenient manner in the manufacture of peroxid colors, (or dyes,) glass, and other substances. It is essential, however, to note (a fact already alluded to) that these compounds may be at a very small cost, indeed, restored to the metallic state by coal, hydrogen, water-gas, or other reducing mediums—such as natural sulfids, (galena or iron pyrites, for example,) preferably sulfids or pyrites containing gold or silver—and the lead may then be employed over again in the constant-circulation process as anodes.

Supposing it is desired to reduce to the metallic state from its oxid two hundred and six kilograms of lead, six kilograms of carbon will suffice to effect the reduction. Similarly chlorid of lead (and also chlorid of copper) may be reduced to the metallic state by means of hydrogen or water-gas or organic substances, hydrochloric acid being formed at the same time, or free chlorin, if air be suitably admitted. This hydrochloric acid and chlorin, as well as sulfurous or sulfuric acid, obtainable from the decomposition of chlorid or of sulfate or of sulfite of lead can be used over and over again for dissolving metallic oxids, such as zinc oxid, and for regenerating the original solutions, for instance, of zinc. In a similar manner it is possible to make use of the described lead-anode process for obtaining also other metals by this electrolytic process—such, for example, as nickel, manganese, chromium, and even alkaline metals or alloys or amalgams of the same, which are more electropositive than lead. On the other hand, this process is also available for the production of metals which are more electronegative—for example, silver, copper, bismuth, iron, or the like, all of which may be obtained from their corresponding solutions. In this latter case a diaphragm is not absolutely necessary.

In the operation last described the lead, as in the extraction of zinc previously described, will likewise be separated from its solution—as, for instance, by means of compounds of the corresponding metal to be obtained, and more particularly by means of sulfates, sulfites, chromates, chlorids, and oxids, and thereby at the same time to maintain a uniform concentration of the metal contents of the lye. In all these cases the lead will constitute an excellent energy-saving or volt-saving anode capable of reducing the electromotive force at the pole by nearly two volts and enabling its salts to be very

readily and reliably separated again, while at the same time, being readily fusible, it permits the metal to be regenerated in a very economical manner and in a solid or granulated state and renders the employment of complicated filtering-machines in the precipitating process unnecessary, inasmuch as the compounds of the lead are as heavy and readily settle as they are precipitated. Lastly, the silver contained in argentiferous lead, (silver lead bullion,) if such be used for the anode, can be readily and completely extracted, since it remains undissolved while the lead is being dissolved and separated.

Similarly to lead, mercury, though it is much more expensive, may be utilized as an anode, inasmuch as it is still more readily recoverable as a metal from its components than lead is; but although lead appears to be the best and most economical material for forming anodes which permit a considerable amount of electric energy to be saved and are at the same time capable of being readily regenerated, yet in some cases, especially where it is desirable that the anode be of small specific weight, other substances may be employed as substitutes for lead. Among these may be instanced, especially, copper. In that case also, however, it is absolutely necessary to prevent the anode solution from becoming too richly impregnated with the metal dissolved therein. This anode solution, which where the anodes are lead must not of course be a solution of pure sulfate, may in the cases just mentioned—i. e., where copper is used—be a sulfate solution without any inconvenience, since this metal is not insoluble as a sulfate; but in this case also the anode solution should not absorb more than from fifty to seventy-five grams per liter of the dissolved metal. Here also, therefore, the operation should be so conducted that the dissolved metal may be precipitated or displaced by materials which are harmless, more particularly compounds of such metals as shall be obtained electrolytically. The copper may again be separated from the sulfate or chlorid solution obtained at the anode in the form of cuprous chlorid, oxychlorid, oxid, protoxid, or sulfid by any well-known means, preferably by means described in my British Patent No. 18,080 of 1890. In fact, all the well-known methods of precipitating metals may be employed, provided they are capable of removing the metal dissolved at the anodes in a harmless and economical manner.

In many cases it will be sufficient to obtain a precipitate of lead or copper simply by the employment of lime or magnesia, and the salts thus obtained, such as chlorid of calcium, may then be very readily utilized again, for instance, in the production of chlorid of zinc from oxid of zinc or carbonate of zinc—as, for example, described in the specification of British Letters Patent No. 11,724 of 1894.

The employment of energy-saving anodes of lead or copper or other easily-reducible

metals or alloys thereof enables convenient electrolytic baths to be readily constructed and made to operate with a very low electromotive force. It has also already been stated above that energy-saving anodes, especially if the latter be lead, in some cases are capable of yielding a surplus of energy, (like galvanic cells.) This applies more especially to those instances where the electromotive force required for the decomposition of certain fluids is less than the electromotive force set up by the act of dissolving the lead, which amounts to about 1.8 volts. Such is the case, for example, where the salts of copper or silver or solutions of nitrates or nitrites or nitro bodies are decomposed by the aid of lead anodes. Hence it follows that these energy-saving anodes, especially lead, which is insoluble in diluted acids, but may be readily reduced from its compounds, may very advantageously also be utilized as anodes in galvanic batteries as substitute for zinc, or the zinc consumed in galvanic batteries may be regenerated by the use of anodes of lead.

The aim to which the process herein described mainly tends is to enable coal or other cheap fuel to be indirectly used in making anodes for saving or producing electricity, or, in other words, to take advantage of the chemical energy inherent in carbon in carrying out electrolytical operations by using anodes which are readily and economically reducible to the metallic state by the action of coal or water-gas or the like.

The dynamic production of electricity has only hitherto utilized about ten per cent. of the energy inherent in carbon, whereas the present process enables a far greater proportion of the energy thus generated to be satisfactorily turned to account. Two-thirds to three-fourths of the electromotive force necessary for chemical decompositions can henceforward be supplied by direct transformation of chemical into electrical energy.

Carbon for itself when directly transformed by electrolysis into oxid of carbon is not capable of furnishing more than .75 volt, whereas by the herein-described system it furnishes indirectly about two volts. Coal, moreover, has the drawback of being a non-conductor of electricity, whereas its "substitute and product," the lead, is a good one. Lastly, conforming to this process, besides coal other sources of energy hitherto completely neglected, such as pyrites or galena, can be utilized.

Having thus described my invention, what I claim as new therein, and desire to secure by Letters Patent, is—

1. A process which consists in placing a soluble metallic anode in a solution of a salt capable of dissolving the same, placing a suitable cathode in a second solution containing a metal other than that contained in the anode solution, separating the two solutions by a suitable diaphragm, passing a current, thereby bringing the anode metal into solution and

depositing the cathode metal, precipitating the anode metal from the anode solution and conveying the resulting solution to the cathode-compartment, substantially as described. 70

2. A process which consists in placing a soluble metallic anode in a solution of a salt capable of dissolving the same, placing a suitable cathode in a second solution containing a metal other than that contained in the anode solution, separating the two solutions by means of a suitable diaphragm, passing a current, thereby bringing the anode metal into solution and depositing the cathode metal, precipitating the anode metal from the anode solution by means of a cathode metal compound and conveying the resulting solution to the cathode-compartment substantially as described. 80

3. A process which consists in placing a metallic anode other than zinc in a solution capable of dissolving the same, placing a suitable cathode in a solution similar to that at the anode but containing also zinc, separating the two solutions by means of a suitable diaphragm, passing a current, thereby bringing the anode metal into solution, and depositing zinc precipitating the anode metal by means of a zinc compound and conveying the resulting solution to the cathode-compartment, substantially as described. 90

4. A process which consists in placing a lead or copper anode in a solution capable of dissolving the same, placing a suitable cathode in a solution similar to that at the anode but containing also zinc, separating the two solutions by a suitable diaphragm, passing a current from the anode through both solutions to the cathode, thereby bringing lead or copper into solution at the anode and depositing zinc at the cathode, precipitating the lead or copper dissolved in the anode solution by adding a zinc compound thereto, and conveying the resulting solution to the cathode-compartment, substantially as set forth. 100

5. A process which consists in placing a lead or copper anode in a solution capable of dissolving the same, placing a suitable cathode in a solution similar to that at the anode but containing also zinc, separating the two solutions by a suitable diaphragm, maintaining their temperature above normal, passing a current from the anode through both solutions to the cathode, thereby bringing the lead or copper into solution at the anode, and depositing the zinc at the cathode, precipitating the lead outside the cells by cooling, and conveying the solution to the cathode-cell, substantially as set forth. 110

6. A process which consists in placing a lead or copper anode in a solution capable of dissolving the same, placing a suitable cathode in a solution similar to that at the anode but containing also zinc, separating the two solutions by a suitable diaphragm, maintaining their temperature above normal, passing a current from the anode through both solutions to the cathode, thereby bringing the lead 120

or copper into solution at the anode, and depositing the zinc at the cathode, precipitating the lead by means of zinc carbonate outside the cells and conveying the resulting solution 5 to the cathode-cell, substantially as set forth.

7. A process which consists in placing a lead or copper anode in a solution capable of dissolving the same, placing a suitable cathode in a solution similar to that at the anode but 10 containing also zinc, separating the two solutions by a suitable diaphragm, maintaining their temperature above normal, passing a current from the anode through both solutions to the cathode, thereby bringing the lead or copper into solution at the anode and 15 depositing zinc at the cathode, precipitating the zinc at the cathode, precipitating the lead by means of zinc oxide and carbonic acid and conveying the resulting solution to the cathode-cells, substantially as set forth.

8. A process which consists in placing a lead 20 or copper anode in a solution capable of dissolving the same, placing a suitable cathode in a solution similar to that at the anode but containing also zinc, separating the two solutions by a suitable diaphragm, maintaining 25 their temperature above normal, passing a current from the anode through both solutions to the cathode, thereby bringing the lead or copper into solution at the anode and depositing zinc at the cathode, recovering the 30 lead, treating a raw material containing zinc with the said solution, and conveying the resulting solution to the cathode-cell, substantially as set forth.

CARL HOEPFNER.

Witnesses:

W. HAUPT,  
E. STEFFAHNY.